

No. 832,738.

PATENTED OCT. 9, 1906.

W. KEMP.

## PROCESS OF SMELTING COPPER MATTE.

APPLICATION FILED OCT. 3, 1903.



**WITNESSES:**

Edward Thorpe  
Walton Harrison

**INVENTOR**

William Kemp

BY

Mem

**ATTORNEYS**

# UNITED STATES PATENT OFFICE.

WILLIAM KEMP, OF TUCSON, ARIZONA TERRITORY, ASSIGNOR, BY DIRECT AND MESNE ASSIGNMENTS, TO THE KEMP HYDRO-CARBON FURNACE COMPANY, A CORPORATION OF NEW YORK.

## PROCESS OF SMELTING COPPER MATTE.

No. 832,738.

Specification of Letters Patent.

Patented Oct. 9, 1906.

Application filed October 3, 1903. Serial No. 175,584.

*To all whom it may concern:*

Be it known that I, WILLIAM KEMP, a citizen of the United States, and a resident of Tucson, in the county of Pima and Territory 5 of Arizona, have invented new and useful Improvements in Processes for Smelting Copper Matte, of which the following is a full, clear, and exact description.

My invention relates to smelting, and more 10 particularly to a process for smelting copper matte so as to produce black or metallic copper directly therefrom.

Reference is to be had to the accompanying drawings, forming a part of this specification, in which similar characters of reference indicate corresponding parts in both the figures.

Figure 1 represents a vertical cross-section through a furnace used for carrying out my 20 process; and Fig. 2 represents a vertical fragmentary section through the lower part of the furnace, taken on the line 2 2 in Fig. 1.

Upon the base 1 is mounted the brickwork 2, from which extend upwardly the walls 3, 25 each wall being preferably thinner at its top than at its bottom. A water-jacket is shown at 4, and the water contained therein is shown at 5. Surmounting this water-jacket is another water-jacket 6, filled with water 7. At 30 8 are shown the oblique openings directly through the walls of the water-jacket 4. The burner-casings are shown at 9 and are supported upon brace-rods 10, and the air-pipes are shown at 11 12, the concentric members 35 of the burner at 13, a cylinder at 14 for supplying to the members 13 an admixture of vapor and steam, a hand-wheel at 15, a clamp at 16, a sight-opening at 18, and a cover therefor at 17, a mixing-tube at 19, and a steam-pipe at 20. This pipe 20 is connected by another pipe 21 with the pipes 22 23, whereby steam is supplied through the mixing-tube 19 from any suitable source. An oil-tube is shown at 24 and is connected with pipes 25 40 26, whereby hydrocarbon oil is supplied to the mixing-tube 19 also from any suitable source. The tap-hole for copper is shown at 27, (see Fig. 2,) and the slag is tapped off from the tap-hole 27<sup>a</sup>. The lower part of the furnace, consisting of the brickwork 2 and wall 3, 45 constitutes the metal-well of the furnace.

The construction of the furnace, the burner, and the mixing-tube form no part of the in-

vention and are fully described in my other applications, Serial Nos. 145,317 and 175,582, 55 filed concurrently herewith. It will be observed, however, that due to the particular construction of the lower part of the furnace herein shown the burner devices are given a downward and inward inclination, the purpose of which will be fully understood from the description hereinafter following.

In explanation of my improved process it may be stated that the copper matte is charged into the furnace in a hard state or 65 condition, with the lowermost stratum or zone thereof resting upon the brickwork 2, the mass of the charge extending or piling upwardly within the smelting-chamber and extending into the stack of the furnace, 70 through which the charging is effected from above in any well-known way, a suitable percentage of flux, as silica, being continuously mixed with the matte during the charging of the matte into the furnace. A burning flame 75 of oil-vapor, steam, and air is continuously forced or projected from the burner devices into or through the mass of the matte at the bottom, the power of the flame being very great, (and approximating 1,200° centigrade,) 80 due to the large excess of air present therein, from pipes 11 and 12 via the casing or windbox 9, the relative diameter of each of said pipes being comparatively large, as shown. The action of said flame is to successively reduce the lowermost strata or zones of the matte to a molten condition, the mass of the matte above being at the same time subjected to a gradual roasting action upwardly, resulting from the fact that the burning mixture takes an upward course through the matte. As each lowermost stratum or zone 85 of the matte is reduced to the proper state of fusion the copper and slag are drawn off through the outlets therefor, the next succeeding and highly-roasted stratum or zone taking its place, and so on continuously as the charging of the matte into the furnace is carried on, it being understood that the desulfurizing of the mass of the matte takes 90 place simultaneously with the reducing action above set forth.

The copper matte is a sulfid of copper and iron and usually contains about fifty per cent. of copper, twenty-four per cent. of sul- 105 fur, and twenty-six per cent. of iron. With

a matte of this composition about fifteen per cent., by weight, of silica, preferably in the form of quartz, is admixed each time the furnace is charged. The chemical reactions of smelting the matte on this basis are shown by the following equations:



The copper matte being a sulfid of copper and iron thus unites with an excess of oxygen supplied by the flame, thereby forming metallic copper, ferrous oxid, and sulfurous-acid gas. Thereupon a second reaction takes place as follows:



that is to say, the ferrous oxid combines with the silica, forming a ferrous silicate or slag, the metallic copper being unchanged by this second reaction. It will thus be seen that the chemical reactions are very simple and that in smelting sulfids the action is one of oxidizing and not of reducing, as would be the case in the ordinary coke-furnace.

25 The process essentially consists of a roasting and a smelting action at the same moment and is attained without previous roasting or fusing of the matte and without the use of coke, coal, charcoal, or other form of 30 free carbon. Neither is it necessary in my process to employ silicious linings or converting plants of any kind. Suppose now that the furnace contains a charge of silica or silicious ore, the quantity of the latter being 35 so apportioned as to take up the iron contents of the matte, and that the flame is turned on, as above described. The flame being forced through the mass of matte and silica immediately attacks the sulfids contained within the matte, thereby forming sulfurous-acid gas. The iron contained within the matte unites with the oxygen in the air, thereby forming ferrous oxid, and the metallic copper in a molten state is thus set 45 free. The sulfurous-acid gas escapes, and the ferrous oxid combines with the silica, forming a liquid slag, which flows off, and the copper being in a molten state and being 50 heavy accumulates in the metal-well, where it is protected against further action of the flame. The slag and copper are tapped off at intervals, as will be readily understood by persons accustomed to handling molten metal. The charging of the matte and silica 55 into the furnace is accomplished in substantially the same manner as the charging of other ores in ordinary smelting processes.

By my process above described copper matte can be smelted so as to produce black 60 copper in one continuous process, beginning with the matte and ending with the metallic copper. The process readily saves seventy-five per cent. of the cost of the process ordinarily used in converting. My process is of 65 peculiar value to smelters who work on small

scale and who at present find it necessary to ship the so-called "fifty-per-cent. matte." My process, in effect, does at a single operation the work otherwise required to first produce a fifty-per-cent. copper matte from raw sulfid ore and then to smelt the matte and produce therefrom metallic copper ready for commercial use.

I desire to state that in the carrying out of my process the use of steam is not altogether 75 essential, though preferably employed in some instances, since substantially the same results may be derived from a flame produced from oil-vapor and air alone, the air being in excess. On the other hand, good 80 results may also be obtained by flame resulting from oil-vapor and steam alone.

Having thus described my invention, I claim as new and desire to secure by Letters Patent—

85 1. The method herein described of producing metallic copper directly from copper matte, which consists in subjecting the matte, while in hard condition, and in the presence of a flux, to the melting action of the flame of 90 a burning mixture of oil-vapor, steam and air.

2. The method herein described of producing metallic copper directly from copper matte, which consists in charging the matte 95 into a furnace in a hard condition, successively fusing the lowermost zones of the matte from the bottom, and desulfurizing the charge.

3. The method herein described of producing metallic copper directly from copper matte, which consists in charging the matte into a furnace in a hard condition, and mixed 100 with a flux, and successively fusing the lowermost zones of the matte from the bottom, 105 and desulfurizing the charge.

4. The method herein described of producing metallic copper direct from copper matte, which consists in charging the matte into a furnace in hard condition and successively 110 subjecting the lowermost zones thereof to the action of an oxidizing and desulfurizing flame.

5. The method herein described of producing metallic copper direct from copper matte, 115 which consists in charging the matte into a furnace in hard condition and successively subjecting the lowermost zones thereof to the action of an oxidizing and desulfurizing flame in the presence of a flux.

6. The method herein described of producing metallic copper direct from copper matte, which consists in charging the matte into a furnace in hard condition and successively 120 subjecting the lowermost zones thereof to the action of an oxidizing and desulfurizing flame in the presence of silica.

7. The method herein described of producing metallic copper direct from copper matte, 125 which consists in charging the matte into a 130

furnace in hard condition and successively subjecting the lowermost zones thereof to the action of a burning mixture in which there is an excess of oxygen.

5 8. The method herein described of producing metallic copper direct from copper matte, which consists in charging the matte into a furnace in hard condition and successively subjecting the lowermost zones thereof to the 10 action of a burning mixture in the presence of a flux and in which there is an excess of oxygen.

9. The method herein described of producing metallic copper direct from copper matte, 15 which consists in charging the matte into a furnace in hard condition, and successively melting the lowermost zones thereof, while oxidizing and desulfurizing the same.

10. The method herein described of producing metallic copper direct from copper 20

matte, which consists in charging the matte into a furnace in hard condition, and successively melting the lowermost zones thereof, while oxidizing and desulfurizing the same, and drawing off the copper from time to 25 time.

11. The method herein described of producing metallic copper direct from copper matte, which consists in charging the matte into a furnace in hard condition, and success- 30 sively melting the lowermost zones thereof, while oxidizing and desulfurizing the same.

In testimony whereof I have signed my name to this specification in the presence of two subscribing witnesses.

WILLIAM KEMP.

Witnesses:

L. W. WAKEFIELD,  
HARRY L. HEFFNER.